



US005565313A

**United States Patent**

[19]

**Ishidai et al.****Patent Number:** **5,565,313****Date of Patent:** **Oct. 15, 1996**[54] **SILVER HALIDE COLOR PHOTOGRAPHIC LIGHT-SENSITIVE MATERIAL**[75] Inventors: **Hiroshi Ishidai; Hiroshi Kita; Yutaka Kaneko**, all of Hino, Japan[73] Assignee: **Konica Corporation**, Tokyo, Japan[21] Appl. No.: **612,072**[22] Filed: **Mar. 7, 1996****Related U.S. Application Data**

[63] Continuation of Ser. No. 354,642, Dec. 13, 1994, abandoned.

**Foreign Application Priority Data**

Dec. 20, 1993 [JP] Japan ..... 5-320185

[51] **Int. Cl.<sup>6</sup>** ..... **G03C 7/38**[52] **U.S. Cl.** ..... **430/551; 430/558**[58] **Field of Search** ..... **430/558, 551****References Cited****U.S. PATENT DOCUMENTS**

|           |         |                 |       |         |
|-----------|---------|-----------------|-------|---------|
| 2,600,788 | 6/1952  | Loria et al.    | ..... | 95/6    |
| 2,807,653 | 9/1957  | Filbey et al.   | ..... | 260/619 |
| 3,519,429 | 7/1970  | Lestina         | ..... | 96/100  |
| 3,725,067 | 4/1973  | Bailey et al.   | ..... | 96/56.5 |
| 3,758,309 | 9/1973  | Bailey et al.   | ..... | 96/136  |
| 3,810,761 | 5/1974  | Bailey et al.   | ..... | 96/84 R |
| 5,032,497 | 7/1991  | Nakayama et al. | ..... | 430/558 |
| 5,063,148 | 11/1991 | Sugita et al.   | ..... | 430/558 |
| 5,104,782 | 4/1992  | Seto et al.     | ..... | 430/558 |
| 5,254,451 | 10/1993 | Kita et al.     | ..... | 430/558 |

**FOREIGN PATENT DOCUMENTS**

|          |        |       |   |
|----------|--------|-------|---|
| 5-241283 | 9/1993 | Japan | . |
| 5-241287 | 9/1993 | Japan | . |

*Primary Examiner*—Lee C. Wright*Attorney, Agent, or Firm*—Finnegan, Henderson, Farabow, Garrett & Dunner, L.L.P.**ABSTRACT**

Disclosed is a silver halide color photographic light-sensitive material comprising at least one of magenta coupler represented by Formula I or II:



wherein R<sup>1</sup> and R<sup>4</sup> each represent a substituent; R<sup>2</sup> and R<sup>3</sup> each represent a substituted or unsubstituted alkyl group; L<sub>1</sub> and L<sub>2</sub> each represent a substituted or unsubstituted alkylene group, an arylene group, an aralkylene group or an arylenealkylene group; Y represents



R<sup>5</sup> and R<sup>6</sup> each represent a substituent; X<sub>1</sub> represents a hydrogen atom or a group capable of splitting off upon reacting with an oxidized product of a color developing agent; Z represents non-metal atomic group forming a 5-membered or 6-membered heterocyclic ring together with a nitrogen atom; m and n each represent an integer of 0 or 1; p represents an integer of 0 to 4; q represents an integer of 0 to 2, provided that when p is 2 or more, R<sup>4</sup> may be the same or different; and each of them may form a ring.

**8 Claims, No Drawings**

## SILVER HALIDE COLOR PHOTOGRAPHIC LIGHT-SENSITIVE MATERIAL

This application is a continuation of application Ser. No. 08/354,642 filed Dec. 13, 1994, now abandoned.

### FIELD OF THE INVENTION

This invention relates to a silver halide color photographic light sensitive material containing a magenta coupler and, particularly, to a silver halide color photographic light sensitive material in which a color reproducibility and color reproducibility can be excellent and a dye image stable against heat and light can be obtained when containing a novel pyrazoloazole type magenta coupler therein.

### BACKGROUND OF THE INVENTION

As for the couplers generally applicable to silver halide color photographic light sensitive materials, there have been known couplers including, for example, the yellow couplers each comprising an open-chained ketomethylene type compound, the magenta couplers each comprising a pyrazolone or pyrazoloazole type compound and the cyan couplers each comprising a phenol or naphthol type compound. Among them, a 5-pyrazolone compound has very often been used for the magenta couplers so far.

The known pyrazolone magenta couplers are described in, for example, U.S. Pat. Nos. 2,600,788 and 3,519,429 and Japanese Patent Publication Open to Public Inspection

The studies and researches have been tried for improving the light-fastness. For example, JP OPI Publication Nos. 59-125732(1984), 61-282845(1986), 61-292639(1986) and 61-279855(1986) disclose the techniques of making combination use of a pyrazoloazole type coupler and a phenol type compound or a phenylether compound and JP OPI Publication Nos. 61-72246(1986), 62-208048(1987), 62-157031(1987) and 63-163351(1988) disclose the techniques of making combination use of a pyrazoloazole type coupler and an amine type compound.

Further, JP OPI Publication No. 63-24256(1988) proposes for a pyrazoloazole type magenta coupler having an alkylloxyphenoxy group.

In the above-given techniques, the light-fastness of magenta dye images are still unsatisfactory and the improvements thereof have been eagerly demanded.

### SUMMARY OF THE INVENTION

This invention has been made for solving the above-mentioned problems. It is, therefore, an object of the invention is to provide a silver halide color photographic light sensitive material excellent in color reproducibility and color developability and remarkably improved in light-fastness of magenta dye images.

The above-mentioned objects can be achieved with a silver halide color photographic light-sensitive material containing at least one kind of a magenta coupler represented by the following Formula [I] or [II]:



Formula [I]



Formula [II]

(hereinafter referred to as JP OPI Publication) Nos. 49-111631(1974) and 57-35858(1982). However, the dyes made of the pyrazolone magenta couplers have produced an undesirable side-absorption which has been demanded for the improvements, as described in 'The Theory of the Photographic Process', the 4th Ed., Macmillan Publishing Co., 1977, pp.356-358; 'Fine Chemical', Vol.14, No.8, CMC Press, pp.38-41; and the Lecture Transcription published at the 1985 Annual convention of the Society of Photographic Science of Japan, pp.108-110.

As described in the above-given literatures, the dyes made of the pyrazoloazole type magenta couplers do not produce any side-absorption. The above-given literatures, U.S. Pat. Nos. 3,725,067, 3,758,309 and 3,810,761 and so forth describe that the couplers of this type are excellent.

However, the light-fastness of azomethine dyes made of the couplers are so seriously low that the characteristics of color photographic light sensitive materials, particularly those of print type color photographic light sensitive materials are seriously spoiled.

wherein R¹ and R⁴ each represent a substituent; R² and R³ each represent a substituted or unsubstituted alkyl group; L¹ and L² each represent a substituted or unsubstituted alkylene group, arylene group, aralkylene group or an arylenealkylene group; Y represents



R⁵ and R⁶ each represent a substituent; X represents a hydrogen atom or a group capable of splitting off upon reaction with an oxidized product of a color developing agent; Z represents a non-metal atomic group forming a 5-membered or 6-membered heterocyclic ring together with a nitrogen atom; m and n represent an integer of 0 or 1; p represents an integer of 0 to 4; q represents an integer of 0 to 2; when p is 2 or more, R⁴ may be the same or different; and each of them may bond each other for forming a ring.

## DETAILED DESCRIPTION OF THE INVENTION

Hereunder, the present invention will be described in detail.

In the above-mentioned Formula [I] and [II], there is no specific limitation for the substituents represented by  $R^1$  and  $R^4$ . Typically, an alkyl group, an aryl group, an anilino group, an acylamino group, a sulfonamido group, an alkylthio group, an arylthio group, an alkenyl group and a cycloalkyl group are cited. In addition, a halogen atom, a cycloalkenyl group, an alkinyl group, a heterocyclic ring, a sulfonyl group, a sulfinyl group, a phosphonyl group, an acyl group, a carbamoyl group, a sulfamoyl group, a cyano group, an alkoxy group, an aryloxy group, a heterocyclic oxy group, a siloxy group, an acyloxy group, a carbamoyloxy group, an amino group, an alkylamino group, an imido group, an ureido group, a sulfamoyl amino group, an alkoxy-carbonylamino group, an aryloxycarbonylamino group, an alkoxy carbonyl group, an aryloxycarbonyl group and a heterocyclic thio group and a spiro compound residual group and a hydrogen carbon residual group having a bridge-head atom are cited.

The alkyl group represented by  $R^1$  and  $R^4$  include preferably, those having 1 to 32 carbons. They may be either straight-chained or branched.

The aryl group represented by  $R^1$  and  $R^4$  includes preferably, a phenyl group.

The acylamino group represented by  $R^1$  and  $R^4$  includes for example, an alkylcarbonylamino group and an arylcarbonylamino group.

The sulfonamide group represented by  $R^1$  and  $R^4$  includes for example, an alkylsulfonylamino group and an arylsulfonylamino group.

An alkyl component and an aryl component in the alkylthio group and the arylthio group represented by  $R^1$  and  $R^4$ , include for example, the above-mentioned alkyl group and aryl group represented by  $R^1$  and  $R^4$ .

The alkenyl group represented by  $R^1$  and  $R^4$  include for example, those having 2 to 32 carbons. The cycloalkyl group includes preferably, those having 3 to 12 carbons, and more preferably those having 5 to 7 carbons. The alkenyl group may be either straight-chained or branched.

The cycloalkenyl group represented by  $R^1$  and  $R^4$  includes preferably, those having 2 to 12 carbons, and more preferably those having 5 to 7 carbons.

The sulfonyl group represented by  $R^1$  and  $R^4$  includes for example, an alkylsulfonyl group and an arylsulfonyl group;

The sulfinyl group includes for example, an alkylsulfinyl group and an arylsulfinyl group.

The phosphonyl group represented by  $R^1$  and  $R^4$  includes for example, an alkylphosphonyl group, alkoxyphosphonyl group, an aryloxyphosphonyl group and an arylphosphonyl group.

The acyl group includes for example, an alkylcarbonyl group and an arylcarbonyl group.

The carbamoyl group includes for example, an alkylcarbamoyl group and an arylsulfamoyl group.

The sulfamoyl group includes for example, an alkylsulfamoyl group and an arylsulfamoyl group.

The acyloxy group includes for example, an alkylcarbonyloxy group and an arylcarbonyloxy group.

The carbamoyloxy group includes for example, an alkylcarbamoyloxy group and an arylcarbamoyloxy group.

The ureido group includes for example, an alkylureido group and an arylureido group.

The sulfamoylamino group includes for example, an alkylsulfamoylamino group and an alkylsulfamoylamino group.

The heterocyclic ring includes preferably, those having a 5-membered to 7-membered group, practically including a 2-furyl group, a 2-thienyl group, a 2-pyrimidinyl group and a 2-benzothiazolyl group.

The heterocyclic oxy group includes preferably, those having 5-membered through 7-membered heterocyclic ring, for example, a 3,4,5,6-tetrahydropyran-2-oxy group and a 1-phenyltetrazole-5-oxy group.

The heterocyclic thio group includes preferably, those having 5-membered through 7-membered heterocyclic thio group including, for example, a 2-pyridylthio group, a 2-benzothiazolylthio group and a 2,4-diphenoxyl-1,3,5-triazole-6-thio group.

The siloxy group includes for example, a trimethylsiloxy group, a triethylsiloxy group and a dimethylbutylsiloxy group.

The imido group includes for example, a succinic acid imido group, a 3-heptadecylsuccinic acid imido group, a phthalic imido group and a glutaric imido group.

The spiro compound residual group includes for example, a spiro[3,3]heptane-1-yl; and

The bridge-having hydrogen carbon residual group having a bridge-head atom includes for example, a bicyclo[2.2.1]heptane-1-yl group, a tricyclo[3.3.1.1<sup>3,7</sup>]decane-1-yl, 7,7-dimethyl-bicyclo[2.2.1]heptane-1-yl.

Each group represented by  $R_1$  and  $R_{14}$ , in addition, includes those having a substituent.

In the above-mentioned Formulas [I] and [II], as a group capable of splitting off upon reaction with an oxidized product of a color developing agent represented by  $X$  include, for example, a halogen atom (chlorine, bromine and fluorine), an alkoxy group, an aryloxy group, a heterocyclic oxy group, an acyloxy group, a sulfonyloxy group, an alkoxy carbonyloxy group, an aryloxycarbonyloxy group, an alkyloxalyloxy group, an alkoxyoxalyloxy group, an alkylthio group, an arylthio group, a heterocyclic thio group, an alkyloxythiocarbonylthio group, an acylamino group, a sulfonamido group, a nitrogen-containing heterocyclic ring bonded with a nitrogen atom, an alkylcarbonylamino group, an aryloxycarbonylamino group and a carboxyl group. Among them, a chlorine atom is particularly preferable.

In addition, an oligomeric coupler such as a dimeric coupler containing a pyrazolotriazole ring in  $X$  and a polymer coupler are included in the present invention.

$R^2$  and  $R^3$  in the above-mentioned Formula [I] and [II] each represent an alkyl group having 1 to 32 carbons, and said alkyl group may be straight-chained or branched, and include for example, a methyl group and an ethyl group, isopropyl group and a hexyl group.

The alkylene group represented by  $L_1$  and  $L_2$  in the above-mentioned Formulas [I] and [II] includes, for example, a methylene group, an ethylene group, a methyl-methylene group and a decamethylene group. The arylene group represented by  $L_1$  and  $L_2$  includes, for example, a phenylene group and a naphthylene group. The aralkylene group and the arylalkylene group represented by  $L_1$  and  $L_2$  include the following compounds;



m and n represents an integer of 0 or 1.

In the above-mentioned Formulas [I] and [II],  $R^5$  and  $R^6$  in each group of



represented by Y include the same as those cited in the above-mentioned  $R^1$  and  $R^4$ . q represents an integer of 0 to 2.

5

In the above-mentioned Formulas [I] and [II], a 5-membered to 6-membered heterocyclic ring represented by



may be saturated or unsaturated. These heterocyclic rings may have a substituent represented by the above-mentioned  $R^1$ ,  $R^4$ ,  $R^5$  and  $R^6$ .

The heterocyclic ring represented by



preferably represents



20

Hereunder, the typical examples of the magenta couplers relating to the present invention will be given. However, the present invention shall not be limited thereto.

(1)



(2)



(3)



(4)



(5)



-continued

(6)



(7)



(8)



(9)



(10)



(11)



(12)



(13)



(14)

-continued

(15)



(16)



(17)



(18)



(19)



(20)



(21)



(22)



(23)



-continued

(24)



(25)



(26)



(27)



(28)



(29)



(30)



(31)





(32)



(33)



(34)



(35)



(36)

$$x:y = 50:50$$

(in term of mol ratio)

The above-mentioned pyrazoloazole type magenta couplers relating to the invention can readily be synthesized by the skilled in the art with reference to 'Journal of the Chemical Society', Perkin I, 1977, pp.2047-2052; U.S. Pat. No. 3,725,067; JP OPI Publication Nos. 59-99437(1984), 58- 42045(1983), 59-162548(1984), 59-171956(1984), 60-33552(1985), 60-43659(1985), 60-172982(1985), 60-190779(1985), 61- 189539(1986), 61-241754(1986), 63-163351(1988) and 62- 157031(1987).

The typical synthesizing examples of the above-mentioned pyrazoloazole type magenta couplers relating to the invention will now be given below.

## Synthesis Examples

### Synthesis Examples

## Synthesis Procedures





## &lt;Synthesis of Intermediate (II)&gt;

In 200 ml of chloroform, 118.13 g (1.0 mol) of hydroxypivalic acid (I) was dissolved. To the mixture, 97 ml (1.2 mol) of pyridine was added. In an iced water bath, the mixture was stirred at 5° C. To the resulting solution, 86.35 g (1.1 mol) of acetyl chloride was dropped for 1 hour. After dropping, the solution was stirred for 30 minutes at 5° C. After removing the iced water bath, the solution was stirred for 2 hours at room temperature. The resulting solution was poured into 200 ml of diluted hydrochloric acid subjected to cooling with ice so that the chloroform layer was separated. Then, the solution was washed twice with 200 ml of diluted hydrochloric acid and washed twice with water. After the solution was dried with magnesium sulfate, the chloroform was distilled off under reduced pressure so that white solid was obtained. This white solid was recrystallized with hexane. Thus, 127.3 g (0.795 mol) of white crystallized intermediate (II) was obtained with yield of 79.5%.

## &lt;Synthesis of Intermediate (III)&gt;

In 350 ml of toluene, 66.6 g (0.416 mol) of intermediate (II) was dissolved. To the solution, 90 ml (1.21 mol) of thionyl chloride was added. The mixture was heated and refluxed for 4 hours. Toluene which served as a solvent and excessive thionyl chloride were distilled off under reduced pressure. Thus, 74.0 g (0.414 mol) of fine brownish solid intermediate (III) was obtained at yield of 99.6%.

## &lt;Synthesis of Intermediate (V)&gt;

In 500 ml of acetonitrile, 76.8 g (0.345 mol) of intermediate (IV) was dissolved. To the solution, 74.0 g (0.414 mol) of intermediate (III) was added. The mixture was heated and refluxed for 2 hours. After heating and refluxing, acetonitrile which served as a solvent was distilled off under reduced pressure. To the solution, 500 ml of toluene and 6 ml of sulfuric acid were added. While removing generated water, the mixture was heated and refluxed for 2 hours.

After heating and refluxing, the solvent was distilled off under reduced pressure. To the mixture, 1 liter of ethyl

acetate was added for extraction and 300 ml of sodium hydrogencarbonate aqueous solution was added for neutralization. In addition, the ethyl acetate layer was three times washed with 300 ml of water. Following this, the layer was dried with magnesium sulfate. Ethyl acetate was distilled off under reduced pressure, and 105.2 g of slight brownish oily crude intermediate (V) was obtained.

## &lt;Synthesis of Intermediate (VI)&gt;

To 105.2 g of crude intermediate (V), 600 ml of acetic anhydride was added. After the solution was heated and refluxed for 2 hours, heating and refluxing were continued while removing excessive acetic anhydride. After removing, the resulting solution was cooled to room temperature. To the resulting solution, 300 ml of methanol and 80 ml of concentrated hydrochloric acid were added. The mixture was heated and refluxed for 2 hours, and then cooled to room temperature. Precipitated sulfur was filtrated. The filtrated solution was concentrated under reduced pressure. To the

mixture, 500 ml of ethyl acetate was added for extraction and a sodium hydroxide aqueous solution was added for neutralization. The ethyl acetate layer was washed three times with 300 ml of water. Then, the solution was dried with magnesium sulfate. Then, ethyl acetate was distilled off under reduced pressure. Thus, a brownish oily product was obtained. By recrystallizing the compound with acetonitrile, 42.4 g (0.179 mol) of slightly pink crystallized intermediate (VI) was obtained at yield of 51.9% (from intermediate (III)).

## &lt;Synthesis of Intermediate (VII)&gt;

To 300 ml of chloroform, 42.0 g (0.178 mol) of intermediate (VI) was dissolved. In an iced water bath, the mixture was stirred at 5° C. To the solution, 22.7 g (0.17 mol) of N-chlorosuccinic acid imide was added gradually for 2 hours. After stirring and addition, the resulting solution was washed three times with 200 ml of water. Following this, the resulting solution was dried with magnesium sulfate, and

then, the solvent was distilled off under reduced pressure. The resulting product was recrystallized with a mixed solvent of ethyl acetate and hexane. Thus, 42.0 g (0.155 mol) of white crystallized intermediate (VII) was obtained at yield of 87.7%.

<Synthesis of Exemplified Compound (I)>

To 500 ml of toluene, 151.4 g (0.341 mol) of intermediate (VIII) described in Japanese Patent O.P.I. Publication No. 224369/1993, 10 g of p-toluene sulfonic acid monohydrate and 42.0 g (0.155 mol) of intermediate (VII) were added. While removing water produced, the mixture was heated and refluxed for 8 hours. The resulting solution was washed with 300 ml of water, 300 ml of diluted hydrochloric acid, 300 ml of an sodium hydrogencarbonate aqueous solution and 300 ml of water in this order. Following this, the solution was dried with magnesium sulfate, and the solvent was distilled off under reduced pressure. The resulting product was recrystallized with a mixed solvent of ethyl acetate and hexane so that 76.4 g (0.113 mol) of white solid Exemplified compound (1) was obtained with yield of 72.6%.

Each structure of intermediates and Exemplified compound (1) were confirmed by <sup>1</sup>H NMR, FD mass-spectral analysis and IR spectral analysis.

It is preferred to contain a magenta coupler applicable to the invention in a silver halide emulsion. The magenta coupler may be contained therein in a well-known method. For example, the magenta coupler relating to the invention can be contained in a silver halide emulsion in the following manner. The magenta coupler relating to the invention is dissolved in a high boiling organic solvent having a boiling point of not lower than 175° C. such as tricresyl phosphate and dibutyl phthalate or a low boiling solvent such as ethyl acetate and butyl propionate independently or, if required, in the mixture thereof independently or in combination, and the resulting solution is mixed with an aqueous gelatin solution containing a surfactant. After that, the resulting mixture is emulsified by making use of a high-speed rotary mixer or a colloid-mill and the emulsified mixture is then added into the silver halide emulsion.

The magenta coupler relating to the invention may usually be used in an amount within the range of  $1 \times 10^{-3}$  to 1 mol and, preferably,  $1 \times 10^{-2}$  to  $8 \times 10^{-1}$  mols per mol of silver halide.

It is also allowed to use the magenta couplers relating to the invention with other kinds of magenta couplers in combination.

It is further allowed to use the magenta couplers relating to the invention with an image stabilizer represented by the following Formula [A] or [B] in combination.



wherein R<sub>21</sub> represents a hydrogen atom, an alkyl group, an alkenyl group, an aryl group or a heterocyclic group.

Among them, the alkyl groups include, for example, the straight-chained or branched alkyl groups such as those of a methyl group, an ethyl group, a propyl group, an n-octyl group, a tert-octyl group, a benzyl group and a hexadecyl group.

The alkenyl groups represented by R<sub>21</sub> include, for example, an allyl group, a hexenyl group and an octenyl group.

The aryl groups represented by R<sub>21</sub> include, for example, a phenyl group and a naphthyl group.

The heterocyclic groups represented by R<sub>21</sub> include, typically, a tetrahydropyran group and a pyrimidyl group.

Each of the groups represented by R<sub>21</sub> include those having a substituent.

In Formula [A], R<sub>22</sub>, R<sub>23</sub>, R<sub>25</sub> and R<sub>26</sub> represent each a hydrogen atom, a halogen atom, a hydroxyl group, an alkyl group, an alkenyl group, an aryl group, an alkoxy group or an acylamino group. Among them, the alkyl, alkenyl and aryl groups include each the same alkyl, alkenyl and aryl groups described of R<sub>21</sub>.

The above-mentioned halogen atoms include a fluorine atom, a chlorine atom and a bromine atom.

The above-mentioned alkoxy groups include, typically, a methoxy group, an ethoxy group and a benzyloxy group.

Further, the acylamino group is represented by R<sub>27</sub>—CONH— in which R<sub>27</sub> represents an alkyl group (such as a methyl, ethyl, n-propyl, n-butyl, n-octyl, tert-octyl or benzyl group), an alkenyl group (such as an allyl, octenyl or oleyl group), an aryl group (such as a phenyl, methoxyphenyl or naphthyl group) or a heterocyclic group (such as a pyridinyl or pyrimidyl group).

In the foregoing Formula [A], R<sub>24</sub> represents an alkyl group, a hydroxyl group, an aryl group, an alkoxy group, an alkenyloxy group or an aryloxy group. Among them, the alkyl and aryl groups include, typically, the same alkyl and aryl groups represented by the foregoing R<sub>21</sub>. And, the alkoxy groups represented by R<sub>24</sub> include the same alkoxy groups described of the foregoing R<sub>22</sub>, R<sub>23</sub>, R<sub>25</sub> and R<sub>26</sub>.

In addition, R<sub>21</sub> and R<sub>22</sub> may be closed in a ring so as to form a 5- or 6-membered heterocyclic ring, and R<sub>23</sub> and R<sub>24</sub> may be closed in a ring so as to form a 5-membered ring. These rings also include those spiro-bonded to other rings.

The typical examples of the compounds represented by the foregoing Formula [A] will now be given below. It is, however, to be understood that the invention shall not be limited thereto.





21

-continued



The compounds represented by Formula [A] can readily be synthesized in the procedures described in, for example, 'Journal of the Chemical Society', 1962, pp.415-417; *ibid.*, 1965, pp.2904 to 2914; 'The Journal of Organic Chemistry', Vol.23, pp.75-76; 'Tetrahedron', Vol.26, 1970, pp.4743-4751; 'Chemical Letter', (4), 1972, pp.315-316; 'Bulletin of Chemical Society of Japan' No.10, 1972, pp.1987-1990; and 'Bulletin of Chemical Society of Japan', Vol.53, 1980, pp.555-556.



Formula [B]

50

wherein R<sub>31</sub> represents a secondary or tertiary alkyl group, a secondary or tertiary alkenyl group, a cycloalkyl group or an aryl group; R<sub>32</sub> represents a halogen atom, an alkyl group, an alkenyl group, a cycloalkyl group or an aryl group; and n<sup>2</sup> is an integer of 0 to 3; provided, when two or more each of R<sub>31</sub> and R<sub>32</sub> are made present, they may be the same with or the different from each other.

Y represents S, SO, SO<sub>2</sub> or an alkylene group.

The secondary or tertiary alkyl groups or the secondary or tertiary alkenyl groups each represented by R<sub>31</sub> include desirably, those having 3 to 32 carbon atoms and, preferably,

22

those having 4 to 12 carbon atoms. They include, typically, a t-butyl, s-butyl, t-amyl, s-amyl, t-octyl, i-propyl, i-propenyl or 2-hexenyl group.

5 The alkyl groups represented by R<sub>32</sub> include, preferably, those having 1 to 32 carbon atoms. The alkenyl groups represented by R<sub>32</sub> include, preferably, those having 2 to 32 carbon atoms. These groups may be straight-chained or branched and they include, typically, a methyl, ethyl, t-butyl, pentadecyl, 1-hexanonyl, 2-chlorobutyl, benzyl, 2,4-di-t-amylphenoxyethyl, 1-ethoxytridecyl, allyl or isopropenyl group.

15 The cycloalkyl groups represented by R<sub>31</sub> and R<sub>32</sub> include, preferably, those having 3 to 12 carbon atoms. They include, typically, a cyclohexyl, 1-methylcyclohexyl or cyclopentyl group.

20 The aryl groups represented by R<sub>31</sub> and R<sub>32</sub> include, preferably, a phenyl group and a naphthyl group. They include, typically, a phenyl, 4-nitrophenyl, 4-t-butylphenyl, 2,4-di-t-amylphenyl, 3-hexadecyloxyphenyl or  $\alpha$ -naphthyl group.

25 The alkylene groups represented by Y<sub>1</sub> include, preferably, those having 1 to 12 carbon atoms. They include, typically, a methylene, ethylene, propylene or hexamethylene group.

30 Each of the groups represented by the above-mentioned R<sub>31</sub>, R<sub>32</sub> and Y<sub>1</sub> are each also allowed to have a substituent.

35 The substituents R<sub>31</sub>, R<sub>32</sub> and Y<sub>1</sub> are each allowed to have include, for example, a halogen atom and a nitro, cyano, sulfonamido, alkoxy, aryloxy, alkylthio, arylthio or acyl group.

40 The typical examples of the compounds represented by Formula [B] will be given below. It is, however, to be understood that the invention shall not be limited thereto.



## 23

-continued



## 24

-continued

B-12



B-5

5

B-6

10

B-7

15

20

25

B-8

30

B-9

35

40

B-10

45

50

B-11

55

56

60

The compounds represented by Formula [B] can readily be synthesized in the procedures described in, for example, U.S. Pat. No. 2,807,653, 'Journal of the Chemical Society', Perkin I, 1979, p.1712.

The image stabilizers represented by the foregoing Formulas [A] and [B] may be used in an amount within the range of, desirably, 5 to 400 mol % and, preferably, 10 to 250 mol % of the pyrazoloazole type magenta couplers relating to the invention.

It is preferable that the pyrazoloazole type magenta couplers of the invention and the above-mentioned image stabilizers are used in one and the same layer. It is, however, allowed to use the image stabilizers in the layer adjacent to a layer containing the above-mentioned couplers.

The silver halides preferably used in the invention are comprised of silver chloride, silver chlorobromide or silver chloroiodobromide and, further, they may also be comprised of a combined mixture such as the mixture of silver chloride and silver bromide.

In the silver halide emulsions applicable to the invention, it is allowed to use any one of silver halides such as silver bromide, silver iodobromide, silver iodochloride, silver chlorobromide, silver chloroiodobromide and silver chloride, provided, they can be used in ordinary silver halide emulsions.

The silver halide grains may be either those having the uniform distribution of silver halide compositions inside the grains or those of the core/shell type having the different silver halide compositions between the inside of the grains and the surface layers of the grains.

The silver halide grains may be either those capable of forming a latent image mainly on the surfaces thereof or those capable of forming a latent image mainly inside the grains thereof.

The silver halide grains may be either those having a regular crystal form such as a cube, octahedron or tetradecahedron or those having an irregular crystal form such as a globular or tabular form. It is allowed to use the grains having any ratios of {100} planes to {111} planes.

These grains may also have a mixed crystal form or may be mixed with the grains having various crystal forms.

The silver halide grains applicable thereto are to have a grain size within the range of, desirably, 0.05 to 30  $\mu\text{m}$  and, preferably, 0.1 to 20  $\mu\text{m}$ .

The silver halide emulsions having any grain size distributions may be used. It is, therefore, allowed to use either the emulsions having a wide grain size distribution (hereinafter referred to as 'polydisperse type emulsions') or the independent or mixed emulsions having a narrow grain size distribution (hereinafter referred to as 'monodisperse type

emulsions'). It is, further, allowed to use the mixtures of the polydisperse type and monodisperse type emulsions. The couplers applicable to the invention include a colored coupler capable of displaying a color compensation effect and the compounds capable of releasing a photographically useful fragment such as a development retarder, a development accelerator, a bleach accelerator, a developing agent, a silver halide solvent, a color toner, a layer hardener, a foggant, an antifoggant, a chemical sensitizer, a spectral sensitizer and a desensitizer. Among these compounds, it is also allowed to use the so-called DIR compounds capable of releasing a development retarder in the course of carrying out a development and improving the sharpness and graininess of an image.

The above-mentioned DIR compounds include those containing a retarder directly coupled to the coupling position thereof and those containing a retarder coupled to the coupling position through a divalent group and capable of releasing the retarder either upon intramolecular nucleophilic reaction or upon intramolecular electron-transfer reaction, produced in a group split off upon coupling reaction, (the latter compounds are hereinafter referred to as 'timing DIR compounds'). The retarders applicable thereto include those becoming diffusible upon splitting off and those not having a diffusibility so much, independently or in combination so as to meet the purposes of application.

The above-mentioned couplers are to make a coupling reaction with the oxidized products of an aromatic primary amine developing agent and these couplers may also be used in combination with a colorless coupler not forming any dyes (hereinafter referred to as 'competing coupler') as a dye-forming coupler.

The yellow couplers preferably applicable to the invention include, for example, the well-known acylacetanilide type couplers. Among these couplers, benzoyl acetanilide type and pivaloyl acetanilide type compounds may advantageously be used.

The cyan couplers preferably applicable to the invention include, for example, phenol type and naphthol type couplers.

It is also allowed to use a color-fog inhibitor for the purposes of preventing a color stain, a sharpness deterioration and/or a rough graininess, which may be produced by transferring the oxidized products of an developing agent or an electron transerrer between the emulsion layers of a light sensitive material (i.e., between the same color-sensitive layers and/or between the different color-sensitive layers).

An image stabilizer capable of preventing the deterioration of a dye image may be applied to the light sensitive materials of the invention. The compounds preferably applicable thereto are described in, for example, RD 17643, Article VII-J.

For the purposes of preventing any fog from being produced by a electric discharge generated by frictionally static-charging a light sensitive material and preventing an image from being deteriorated by UV rays, a UV absorbent may also be contained in the hydrophilic colloidal layers thereof such as the protective layers and interlayers.

For the purpose of preventing a magenta-dye forming coupler from being deteriorated by formalin in the course of preserving a light sensitive material, a formalin scavenger may further be used in the light sensitive material.

The invention can preferably be applied to a color negative film, a color paper, a color reversal film and so forth.

Now, the invention will be detailed with reference to the following preferred embodiments. It is, however, to be understood that the embodiments of the invention shall not be limited thereto.

## EXAMPLE 1

Sample 101 of multilayered silver halide color photographic light sensitive materials was prepared in the following manner. Over to a polyethylene-laminated paper support containing polyethylene on one side thereof and titanium oxide on the other side thereof, each of the layers having the compositions shown in the following Tables 1 and 2 were coated thereover on the side of the polyethylene layer containing titanium oxide.

TABLE 1

| 15 | Layer                                   | Composition                                                                                                                                                                                | Coat-<br>ing<br>weight<br>(g/m <sup>2</sup> )                |
|----|-----------------------------------------|--------------------------------------------------------------------------------------------------------------------------------------------------------------------------------------------|--------------------------------------------------------------|
| 20 | 7th layer<br>(Protective<br>layer)      | Gelatin                                                                                                                                                                                    | 1.00                                                         |
|    | 6th layer<br>(UV absorbing<br>layer)    | Gelatin<br>UV absorbent (UV-1)<br>UV absorbent (UV-2)<br>UV absorbent (UV-3)<br>Antistaining agent (HQ-1)<br>DNP<br>PVP<br>Anti-irradiation dye (AIC-1)                                    | 0.40<br>0.10<br>0.04<br>0.16<br>0.01<br>0.20<br>0.03<br>0.02 |
|    | 5th layer<br>(Res-sensitive<br>layer)   | Gelatin<br>Red-sensitive silver chlorobromide<br>emulsion (Em-R)<br>Cyan coupler (EC-1)<br>Cyan coupler (EC-2)<br>Dye-image stabilizer (ST-1)<br>Antistaining agent (HQ-1)<br>HBS-1<br>DOP | 1.30<br>0.21<br>0.24<br>0.08<br>0.20<br>0.01<br>0.20<br>0.20 |
|    | 4th layer<br>(UV absorbing<br>layer)    | Gelatin<br>UV absorbent (UV-1)<br>UV absorbent (UV-2)<br>UV absorbent (UV-3)<br>Antistaining agent (HQ-1)<br>DNP                                                                           | 0.94<br>0.28<br>0.09<br>0.38<br>0.03                         |
|    | 3rd layer<br>(Green-sensitive<br>layer) | Gelatin<br>Green-sensitive silver chlorobromide<br>emulsion (Em-G)<br>Magenta coupler (EM-1)<br>DNP<br>Anti-irradiation dye (AIM-1)                                                        | 1.40<br>0.17<br>0.75*                                        |
|    | 2nd layer<br>(Interlayer)               | Gelatin<br>Antistaining agent (HQ-2)<br>Antistaining agent (HQ-3)<br>Antistaining agent (HQ-4)<br>Antistaining agent (HQ-5)<br>DIDP<br>Antimold (F-1)                                      | 1.20<br>0.03<br>0.03<br>0.05<br>0.23<br>0.06<br>0.002        |
|    |                                         |                                                                                                                                                                                            |                                                              |
|    |                                         |                                                                                                                                                                                            |                                                              |
|    |                                         |                                                                                                                                                                                            |                                                              |
|    |                                         |                                                                                                                                                                                            |                                                              |

TABLE 2

| 55 | Layer                                  | Composition                                                                                                                                                                                                                  | Coat-<br>ing<br>weight<br>(g/m <sup>2</sup> )                |
|----|----------------------------------------|------------------------------------------------------------------------------------------------------------------------------------------------------------------------------------------------------------------------------|--------------------------------------------------------------|
| 60 | 1st layer<br>(Blue-sensitive<br>layer) | Gelatin<br>Blue-sensitive silver chlorobromide<br>emulsion (Em-B)<br>Yellow coupler (EY-1)<br>Dye-image stabilizer (ST-1)<br>Dye-image stabilizer (ST-2)<br>Antistaining agent (HQ-1)<br>Anti-irradiation dye (AIY-1)<br>DNP | 1.20<br>0.26<br>0.80<br>0.30<br>0.20<br>0.02<br>0.01<br>0.20 |
|    | Support                                | Polyethylene-laminated paper sheet                                                                                                                                                                                           |                                                              |
|    |                                        |                                                                                                                                                                                                                              |                                                              |
|    |                                        |                                                                                                                                                                                                                              |                                                              |
|    |                                        |                                                                                                                                                                                                                              |                                                              |
|    |                                        |                                                                                                                                                                                                                              |                                                              |
|    |                                        |                                                                                                                                                                                                                              |                                                              |
|    |                                        |                                                                                                                                                                                                                              |                                                              |
|    |                                        |                                                                                                                                                                                                                              |                                                              |
|    |                                        |                                                                                                                                                                                                                              |                                                              |

\*milli-mol/m<sup>2</sup>

Amounts of the silver halide emulsions added were each shown in terms of the silver contents.

The coating solutions were each prepared in the following manner.

Coating Solution for the 1st Layer

Ethyl acetate of 60 cc was added and dissolved into 26.7 g of yellow coupler (EY-1), 10.0 g of dye-image stabilizer (ST-1), 6.67 g of a dye-image stabilizer (ST-2), 0.67 g of antistaining agent (HQ-1) and 6.67 g of high-boiling organic solvent (DNP). The resulting solution was emulsified and dispersed in 220 cc of 10% gelatin aqueous solution containing 7 cc of 20% surfactant (SU-2) aqueous solution by making use of a supersonic homogenizer, so that a yellow coupler dispersed solution could be prepared.

The resulting dispersed solution was mixed with the following blue-sensitive silver halide emulsion (containing

8.67 g of silver) and antiirradiation dye (AIY-1) was further added thereto, so that the coating solution for the 1st layer could be prepared.

The coating solutions for the 2nd through 7th layers were also prepared in the same manner as in the above-mentioned coating solution for the 1st layer. Besides, for the layer hardeners, (HH-1) were each added to the 2nd and 4th layers and (HH-2) to the 7th layer, respectively. For the coating aids, surfactants (SU-1) and (SU-3) were each added thereto so that the surface tension of each layer could be controlled.

The chemical structures of the compounds applied to each of the above-mentioned layers were as follows.



**29**

-continued

**30**

ST-4



(Compounds described in Japanese Patent O.P.I.  
Publication No. 224369/1993)



ST-5

(A compound described in Japanese Patent O.P.I.  
Publication No. 224369/1993)



EM-1



EM-2

(A compound described in Japanese Patent O.P.I.  
Publication No. 67142/1992)



EM-3



UV-1



UV-2



UV-3

DOP = Diethyl phthalate

-continued

DNP = Dinonyl phthalate

DIDP = Diisodecyl phthalate

PVP = Polyvinyl pyrrolidone



HQ-1

HQ-2

HQ-3

HQ-4

HQ-5

HBS-1

AIM-1

AIC-1



Silver halide emulsions used for the 1st layer, the 3rd 35 layer and the 5th layer are as follows:

Blue-Sensitive Silver Halide Emulsion (Em-B)

This was a monodisperse type cubic silver chlorobromide emulsion having an average grain size of 0.85  $\mu\text{m}$ , a variation coefficient of 0.07 and a silver chloride content of 99.5 mol %. 40

|                                               |                                    |
|-----------------------------------------------|------------------------------------|
| Sodium thiosulfate                            | 0.8 mg/mol of AgX                  |
| Chloroauric acid                              | 0.5 mg/mol of AgX                  |
| Stabilizer STAB-1                             | $6 \times 10^{-4}$ mols/mol of AgX |
| Sensitizing dye BS-1                          | $4 \times 10^{-4}$ mols/mol of AgX |
| Sensitizing dye BS-2                          | $1 \times 10^{-4}$ mols/mol of AgX |
| Green-sensitive silver halide emulsion (Em-G) |                                    |

This was a monodisperse type cubic silver chlorobromide emulsion having an average grain size of 0.43  $\mu\text{m}$ , a variation coefficient of 0.08 and a silver chloride content of 99.5 mol %. 50

|                      |                                    |
|----------------------|------------------------------------|
| Sodium thiosulfate   | 1.5 mg/mol of AgX                  |
| Chloroauric acid     | 1.0 mg/mol of AgX                  |
| Stabilizer STAB-1    | $6 \times 10^{-4}$ mols/mol of AgX |
| Sensitizing dye GS-1 | $4 \times 10^{-4}$ mols/mol of AgX |

-continued

Red-sensitive silver halide emulsion (Em-R)

This was a monodisperse type cubic silver chlorobromide emulsion having an average grain size of 0.50  $\mu\text{m}$ , a variation coefficient of 0.08 and a silver chloride content of 99.5 mol %. 40

|                      |                                    |
|----------------------|------------------------------------|
| Sodium thiosulfate   | 1.8 mg/mol of AgX                  |
| Chloroauric acid     | 2.0 mg/mol of AgX                  |
| Stabilizer STAB-1    | $6 \times 10^{-4}$ mols/mol of AgX |
| Sensitizing dye RS-1 | $1 \times 10^{-4}$ mols/mol of AgX |

The chemical structures of the compounds applied to each of the monodisperse type cubic emulsions were as follows.



-continued

(CH<sub>2</sub>)<sub>3</sub>SO<sub>3</sub>H.N(C<sub>2</sub>H<sub>5</sub>)<sub>3</sub>(CH<sub>2</sub>)<sub>3</sub>SO<sub>3</sub>H.N(C<sub>2</sub>H<sub>5</sub>)<sub>3</sub>Br<sup>-</sup>NHCOC<sub>2</sub>H<sub>5</sub>

BS-2

GS-1

RS-1

STAB-1

-continued

Next, Samples 102 through 128 were each prepared in the same manner as in Sample 101, except that the coupler EM-1 of the 3rd layer was replaced by the same mols of the coupler of the invention shown in the following Table-3 and the dye-image stabilizer was replaced by those shown in Table-3, respectively.

The chemical structures of the magenta couplers EM-2, EM-3 and EM-4 each applied to the comparative samples are shown together with the chemical structure of the foregoing EM-1.

The resulting samples were each exposed to green light through a wedge in an ordinary procedures and they were then processed in the following processing steps.

| Processing step  | Temperature    | Time   |
|------------------|----------------|--------|
| Color developing | 35.0 ± 0.3° C. | 45 sec |
| Bleach-fixing    | 35.0 ± 0.5° C. | 45 sec |
| Stabilizing      | 30 to 34° C.   | 90 sec |
| Drying           | 60 to 80° C.   | 60 sec |

The compositions of each of the processing solution will be given below.

The processing solutions were each replenished in an amount of 80 cc per m<sup>2</sup> of a subject silver halide color photographic light sensitive material.

| Color developer            | Tank solution | Replenishing solution |
|----------------------------|---------------|-----------------------|
| Pure water                 | 800 cc        | 800 cc                |
| Triethanol amine           | 10 g          | 18 g                  |
| N,N-diethyl hydroxyl amine | 5 g           | 9 g                   |

35

40

45

50

55

60

65

| Color developer                                                     | Tank solution | Replenishing solution | Color developer                                                                                    | Tank solution | Replenishing solution |
|---------------------------------------------------------------------|---------------|-----------------------|----------------------------------------------------------------------------------------------------|---------------|-----------------------|
| Potassium chloride                                                  | 2.4 g         |                       | 1-hydroxyethylidene-1,1-diphosphonic acid                                                          | 1.0 g         | 1.8 g                 |
| N-ethyl-N-β-methanesulfonamidoethyl-3-methyl-4-aminoaniline sulfate | 5.4 g         | 8.2 g                 | Fluorescent whitening agent, (a 4,4'-diaminostilbene sulfonic acid derivative)                     | 1.0 g         | 1.8 g                 |
| Potassium carbonate                                                 | 27 g          | 27 g                  | Add water to make in total of 1000 cc                                                              |               |                       |
|                                                                     |               |                       |                                                                                                    |               |                       |
|                                                                     |               |                       | Adjust pH values of the tank solution to be 10.0 and of the replenisher to be 10.60, respectively. |               |                       |
|                                                                     |               |                       | Bleach-fixer (The same in both of the tank solution and the replenisher)                           |               |                       |
|                                                                     |               |                       | Ferric ammonium ethylenediamine tetraacetate, dihydrate                                            | 60 g          |                       |
|                                                                     |               |                       | Ethylenediaminetetraacetic acid                                                                    | 3 g           |                       |
|                                                                     |               |                       | Ammonium thiosulfate (in an aqueous 70% solution)                                                  | 100 cc        |                       |
|                                                                     |               |                       | Ammonium sulfite (in an aqueous 40% solution)                                                      | 27.5 cc       |                       |
|                                                                     |               |                       | Add water to make in total of                                                                      | 1000 cc       |                       |
|                                                                     |               |                       | Adjust pH with potassium carbonate or glacial acetic acid to be                                    |               | pH 5.7                |
|                                                                     |               |                       | Stabilizer (The same in both of the tank solution and the replenisher)                             |               |                       |
|                                                                     |               |                       | 5-chloro-2-methyl-4-isothiazoline-3-one                                                            | 1.0 g         |                       |
|                                                                     |               |                       | Ethylene glycol                                                                                    | 1.0 g         |                       |
|                                                                     |               |                       | 1-hydroxyethylidene-1,1-                                                                           | 2.0 g         |                       |

|                                                                               |         |  |  |  |
|-------------------------------------------------------------------------------|---------|--|--|--|
| di-phosphonic acid                                                            |         |  |  |  |
| Ethylenediaminetetraacetic acid                                               | 1.0 g   |  |  |  |
| Ammonium hydroxide (in an aqueous 20% solution)                               | 3.0 g   |  |  |  |
| Fluorescent whitening agent (a 4,4'-diaminostilbene sulfonic acid derivative) | 1.5 g   |  |  |  |
| Add water to make in total of                                                 | 1000 cc |  |  |  |
| Adjust pH with sulfuric acid or potassium hydroxide to be                     | pH 7.0  |  |  |  |

The following evaluation were each carried out by making use of the samples which were continuously processed.  $\langle D_{max} \rangle$

The maximum color densities thereof were measured.

<Light-Fastness>

The resulting samples were each exposed to a Xenon fadometer for 7 days and the dye image residual percentage (%) thereof at the initial density of 1.0 were found out.

The results thereof are shown in Table 3.

TABLE 3

| Sample No. | Magenta coupler in the 3rd layer | Dmax | Dye image residual ratio (%) |
|------------|----------------------------------|------|------------------------------|
| 101 (Comp) | EM-1                             | 1.96 | 32                           |
| 102 (Comp) | EM-2                             | 2.33 | 68                           |
| 103 (Inv)  | (1)                              | 2.47 | 81                           |
| 104 (Inv)  | (2)                              | 2.43 | 73                           |
| 105 (Inv)  | (3)                              | 2.49 | 83                           |
| 106 (Inv)  | (8)                              | 2.44 | 80                           |
| 107 (Inv)  | (24)                             | 2.47 | 85                           |
| 108 (Comp) | EM-3                             | 2.01 | 29                           |
| 109 (Inv)  | (32)                             | 2.36 | 76                           |
| 110 (Inv)  | (34)                             | 2.34 | 75                           |

As is apparent from Table 3, Samples 103 through 107 and Samples 109 through 110 each using the magenta coupler of the present invention is excellent in terms of Dmax and light-fastness due to effects caused by alkyl group branching at the root of the ballast group compared to comparative example Nos. 101, 102 and 108.

## EXAMPLES 1-2

Sample Nos. 111 to 130 were prepared by adding dye image stabilizers as shown in the following Table 4 each having the equivalent mol to that of the magenta coupler in the 3rd layer of Sample No. 101 in Example 1.

By the use of the resulting samples, the same evaluation as Example 1 was conducted. Table 4 shows the results thereof.

TABLE 4

| Sample No  | Magenta coupler in the 3rd layer | Dye image stabilizer | Dmax | Dye image density residual ratio (%) |
|------------|----------------------------------|----------------------|------|--------------------------------------|
| 111 (Comp) | EM-1                             | ST-3, ST-4           | 2.08 | 70                                   |
| 112 (Comp) | EM-1                             | ST-3, ST-4           | 2.04 | 68                                   |
| 113 (Comp) | EM-2                             | ST-4                 | 2.37 | 77                                   |
| 114 (Comp) | EM-2                             | ST-5                 | 2.34 | 76                                   |
| 115 (Inv)  | (1)                              | ST-4                 | 2.49 | 85                                   |
| 116 (Inv)  | (1)                              | ST-5                 | 2.48 | 85                                   |
| 117 (Inv)  | (2)                              | ST-4                 | 2.48 | 82                                   |
| 118 (Inv)  | (2)                              | ST-5                 | 2.48 | 81                                   |
| 119 (Inv)  | (3)                              | ST-4                 | 2.50 | 89                                   |
| 120 (Inv)  | (3)                              | ST-5                 | 2.49 | 86                                   |
| 121 (Inv)  | (8)                              | ST-4                 | 2.45 | 82                                   |
| 122 (Inv)  | (8)                              | ST-5                 | 2.44 | 81                                   |

TABLE 4-continued

| Sample No  | Magenta coupler in the 3rd layer | Dye image stabilizer | Dmax | Dye image density residual ratio (%) |
|------------|----------------------------------|----------------------|------|--------------------------------------|
| 123 (Inv)  | (24)                             | ST-4                 | 2.51 | 88                                   |
| 124 (Inv)  | (24)                             | ST-5                 | 2.50 | 87                                   |
| 125 (Comp) | EM-3                             | ST-3, ST-4           | 2.04 | 69                                   |
| 126 (Comp) | EM-3                             | ST-3, ST-5           | 2.08 | 72                                   |
| 127 (Inv)  | (32)                             | ST-4                 | 2.39 | 78                                   |
| 128 (Inv)  | (32)                             | ST-5                 | 2.41 | 77                                   |
| 129 (Inv)  | (34)                             | ST-4                 | 2.38 | 77                                   |
| 130 (Inv)  | (34)                             | ST-5                 | 2.41 | 78                                   |

As is apparent from Table 4, in the samples wherein the dye image stabilizer is added too, Sample Nos. 115 to 124 and 127 to 130 each using the magenta couplers of the present invention are superior to Comparative example Nos. 111 through 114 and 125 through 126 in terms of Dmax and light-fastness. In addition, when comparing to Sample Nos. 101 through 110 shown in Table 3, it can be understood that both of sensitive property and light-fastness were improved due to the presence of the dye image stabilizer.

## EXAMPLE 3

Reflection spectral light-absorption spectra of Sample Nos. 101 to 110 in Example 1 were measured so that the spectral absorption characteristics were evaluated by means of  $\lambda_{max}$  and Abs.600.

$\lambda_{max}$ : represents the maximum absorption wavelength of a wedge at the reflection optical density of 1.0.

Abs.600: represents the absorption degree at 600 nm of the wedge at the reflection optical density of 1.0.

TABLE 5

| Sample No. | Magenta coupler in the 3rd layer | $\lambda_{max}$ (nm) | Abs. 600 |
|------------|----------------------------------|----------------------|----------|
| 101 (Comp) | EM-1                             | 547                  | 0.44     |
| 102 (Comp) | EM-2                             | 548                  | 0.40     |
| 103 (Inv)  | (1)                              | 548                  | 0.34     |
| 104 (Inv)  | (2)                              | 547                  | 0.35     |
| 105 (Inv)  | (3)                              | 548                  | 0.35     |
| 106 (Inv)  | (8)                              | 549                  | 0.36     |
| 107 (Inv)  | (24)                             | 548                  | 0.34     |
| 108 (Comp) | EM-3                             | 546                  | 0.43     |
| 109 (Inv)  | (32)                             | 547                  | 0.38     |
| 110 (Inv)  | (34)                             | 548                  | 0.39     |

As is apparent from Table 5, in Sample Nos. 103 to 107 and 109 to 110 each employing the magenta coupler of the present invention, the absorption degree at 600 nm was decreased (in other words, absorption has become sharp) compared to Sample Nos. 101, 102 and 108 each using comparative couplers, thus, color reproducibility has been improved.

## EXAMPLE 4

On one side of a triacetylcellulose film support, subbing was provided. On a side opposite to the surface of the support (the reverse surface), layers having the following composition were formed successively in that order from the support side.

Incidentally, the amount added in the silver halide photographic light-sensitive material was described in terms of an amount per 1 m<sup>2</sup>. In addition, silver halide and colloidal

silver were described after being converted to silver.

-continued

Backside surface 1st layer

Aluminasol AS-100 (aluminum oxide)  
(produced by Nissan Kagaku Co. Ltd.)

0.8 g

5

Backside surface 2nd layer

Diacetylcellulose  
Stearic acid

100 mg  
10 mg

Silica fine particle (average particle size is 0.2  $\mu\text{m}$ )

50 mg

1st layer; Anti-halation layer (HC)

|                              |        |
|------------------------------|--------|
| Black colloidal silver       | 0.15 g |
| UV absorber (UV-1)           | 0.20 g |
| Colored cyan coupler (CC-1)  | 0.02 g |
| High boiling solvent (Oil-1) | 0.20 g |
| High boiling solvent (Oil-2) | 0.20 g |
| Gelatin                      | 1.6 g  |

2nd layer; Intermediate layer (IL-1)

|         |       |
|---------|-------|
| Gelatin | 1.3 g |
|---------|-------|

|                                                                                                            |       |
|------------------------------------------------------------------------------------------------------------|-------|
| 3rd layer; Low sensitive red sensitivity emulsion layer (R-L)                                              |       |
| Silver bromoiodide emulsion (average grain size is 0.3 $\mu\text{m}$ (average iodide content is 2.0 mol %) | 0.4 g |
| Silver bromoiodide emulsion (average grain size is 0.4 $\mu\text{m}$ (average iodide content is 8.0 mol %) | 0.3 g |

|                              |                                          |
|------------------------------|------------------------------------------|
| Sensitizing dye (S-1)        | $3.2 \times 10^{-4}$ (mol/mol of silver) |
| Sensitizing dye (S-2)        | $3.2 \times 10^{-4}$ (mol/mol of silver) |
| Sensitizing dye (S-3)        | $0.2 \times 10^{-4}$ (mol/mol of silver) |
| Cyan coupler (C-1)           | 0.50 g                                   |
| Cyan coupler (C-2)           | 0.13 g                                   |
| Colored cyan coupler (CC-1)  | 0.07 g                                   |
| DIR compound (D-1)           | 0.006 g                                  |
| DIR compound (D-2)           | 0.01 g                                   |
| High boiling solvent (Oil-1) | 0.55 g                                   |
| Gelatin                      | 1.0 g                                    |

4th layer; High sensitive red sensitivity emulsion layer (R-H)

|                                                                                                                   |       |
|-------------------------------------------------------------------------------------------------------------------|-------|
| Silver bromoiodide emulsion (average grain size is 0.7 $\mu\text{m}$ (average iodide content amount is 7.5 mol %) | 0.9 g |
|-------------------------------------------------------------------------------------------------------------------|-------|

|                              |                                          |
|------------------------------|------------------------------------------|
| Sensitizing dye (S-1)        | $1.7 \times 10^{-4}$ (mol/mol of silver) |
| Sensitizing dye (S-2)        | $1.6 \times 10^{-4}$ (mol/mol of silver) |
| Sensitizing dye (S-3)        | $0.1 \times 10^{-4}$ (mol/mol of silver) |
| Cyan coupler (C-2)           | 0.23 g                                   |
| Colored cyan coupler (CC-1)  | 0.03 g                                   |
| DIR compound (D-2)           | 0.02 g                                   |
| High boiling solvent (Oil-1) | 0.25 g                                   |
| Gelatin                      | 1.0 g                                    |

5th layer; Intermediate layer (IL-2)

|         |       |
|---------|-------|
| Gelatin | 0.8 g |
|---------|-------|

6th layer; Low sensitive green sensitivity emulsion layer (G-L)

|                                                                                                            |                                          |
|------------------------------------------------------------------------------------------------------------|------------------------------------------|
| Silver bromoiodide emulsion (average grain size is 0.4 $\mu\text{m}$ (average iodide content is 8.0 mol %) | 0.6 g                                    |
| Silver bromoiodide emulsion (average grain size is 0.3 $\mu\text{m}$ (average iodide content is 2.0 mol %) | 0.2 g                                    |
| Sensitizing dye (S-4)                                                                                      | $6.7 \times 10^{-4}$ (mol/mol of silver) |
| Sensitizing dye (S-5)                                                                                      | $0.8 \times 10^{-4}$ (mol/mol of silver) |
| Magenta coupler (M-1)                                                                                      | 0.45 g                                   |
| Colored magenta coupler (CM-1)                                                                             | 0.10 g                                   |
| DIR compound (D-3)                                                                                         | 0.02 g                                   |
| High boiling solvent (Oil-2)                                                                               | 0.7 g                                    |
| Gelatin                                                                                                    | 1.0 g                                    |

7th layer; High sensitive red sensitivity emulsion layer (G-H)

|                                                                                                            |       |
|------------------------------------------------------------------------------------------------------------|-------|
| Silver bromoiodide emulsion (average grain size is 0.7 $\mu\text{m}$ (average iodide content is 7.5 mol %) | 0.9 g |
|------------------------------------------------------------------------------------------------------------|-------|

|                              |                                          |
|------------------------------|------------------------------------------|
| Sensitizing dye (S-6)        | $1.1 \times 10^{-4}$ (mol/mol of silver) |
| Sensitizing dye (S-7)        | $2.0 \times 10^{-4}$ (mol/mol of silver) |
| Sensitizing dye (S-8)        | $0.3 \times 10^{-4}$ (mol/mol of silver) |
| Magenta coupler (M-1)        | 0.35 g                                   |
| Colored cyan coupler (CM-1)  | 0.04 g                                   |
| DIR compound (D-3)           | 0.004 g                                  |
| High boiling solvent (Oil-2) | 0.35 g                                   |
| Gelatin                      | 1.0 g                                    |

8th layer; Yellow filter layer (YC)

|                              |        |
|------------------------------|--------|
| Yellow colloidal layer       | 0.1 g  |
| Additive (HS-1)              | 0.07 g |
| Additive (HS-2)              | 0.07 g |
| Additive (SC-1)              | 0.12 g |
| High boiling solvent (Oil-2) | 0.15 g |
| Gelatin                      | 1.0 g  |

9th layer; Low sensitive blue sensitivity emulsion layer (B-L)

|                                                                                                            |                                          |
|------------------------------------------------------------------------------------------------------------|------------------------------------------|
| Silver bromoiodide emulsion (average grain size is 0.3 $\mu\text{m}$ (average iodide content is 2.0 mol %) | 0.25 g                                   |
| Silver bromoiodide emulsion (average grain size is 0.4 $\mu\text{m}$ (average iodide content is 8.0 mol %) | 0.25 g                                   |
| Sensitizing dye (S-9)                                                                                      | $5.8 \times 10^{-4}$ (mol/mol of silver) |
| Yellow coupler (Y-1)                                                                                       | 0.6 g                                    |
| Yellow coupler (Y-2)                                                                                       | 0.32 g                                   |
| DIR compound (D-1)                                                                                         | 0.003 g                                  |
| DIR compound (D-2)                                                                                         | 0.006 g                                  |
| High boiling solvent (Oil-2)                                                                               | 0.18 g                                   |
| Gelatin                                                                                                    | 1.3 g                                    |

10th layer; High sensitive blue sensitivity emulsion layer (B-H)

|                                                                                                            |                                          |
|------------------------------------------------------------------------------------------------------------|------------------------------------------|
| Silver bromoiodide emulsion (average grain size is 0.8 $\mu\text{m}$ (average iodide content is 8.5 mol %) | 0.5 g                                    |
| Sensitizing dye (S-10)                                                                                     | $3 \times 10^{-4}$ (mol/mol of silver)   |
| Sensitizing dye (S-11)                                                                                     | $1.2 \times 10^{-4}$ (mol/mol of silver) |
| Yellow coupler (Y-1)                                                                                       | 0.18 g                                   |
| Yellow coupler (Y-2)                                                                                       | 0.10 g                                   |
| High boiling solvent (Oil-2)                                                                               | 0.05 g                                   |
| Gelatin                                                                                                    | 1.0 g                                    |

11th layer; 1st protective layer (PRO-1)

|                                                                |        |
|----------------------------------------------------------------|--------|
| Silver bromoiodide (average grain size is 0.08 $\mu\text{m}$ ) | 0.3 g  |
| UV-absorber (UV-1)                                             | 0.07 g |
| UV-absorber (UV-2)                                             | 0.10 g |
| Additive (HS-1)                                                | 0.2 g  |
| Additive (HS-2)                                                | 0.1 g  |
| High boiling solvent (Oil-1)                                   | 0.07 g |
| High boiling solvent (Oil-3)                                   | 0.07 g |
| Gelatin                                                        | 0.8 g  |

12th layer; 2nd protective layer (PRO-2)

|                                                                                                                                            |         |
|--------------------------------------------------------------------------------------------------------------------------------------------|---------|
| Compound A                                                                                                                                 | 0.04 g  |
| Compound B                                                                                                                                 | 0.004 g |
| Polymethylmethacrylate (average particle size is 3 $\mu\text{m}$ )                                                                         | 0.02 g  |
| Copolymer wherein methylmethacrylate: ethylmethacrylate : methacrylic acid = 3:3:4 (by weight) (average particle size is 3 $\mu\text{m}$ ) | 0.13 g  |

Incidentally, the above-mentioned light-sensitive material 101 contains compounds SU-1 and SU-2, a viscosity regulator, hardeners H-1 and H-2, stabilizer ST-1, antifoggants AF-1 and AF-2 (whose weight average molecular weight are respectively 10,000 and 1,100,000), dyes AI-1, AI-2 and DI-1 (9.4 g/m<sup>2</sup>).

The silver bromoiodide emulsion in the 10th layer was 50 prepared by the following method.

With a mono-dispersed silver bromoiodide grain having an average grain size of 0.33  $\mu\text{m}$  (silver iodide content of 2 mol %) as a seed crystal, the silver bromoiodide emulsion was prepared by the use of a double jet method.

While solution <G-1> kept at 70° C., pAg 7.8 and pH 7.0 was stirred completely, the seed emulsion equivalent to 0.34 mol was added thereto.

(Formation of an Inner High Iodide Content Phase—the Shell Phase)

Following the above, while keeping the flow rate ratio of <H-1> to <S-1> at 1:1, addition of the seed emulsion was continued for 86 minutes, in which the flow rate was gradually enhanced (the last flow rate was 3.6 times the initial flow rate).

(Formation of an Outer Low Iodide Content Phase—the Shell Phase)

Following this, while keeping pAg 10.1 and pH 6.0 and the flow rate ratio of <H-2> and <S-2> at 1:1, addition of the seed emulsion was continued for 65 minutes, in which the flow rate was gradually enhanced (the last flow rate was 5.2 times the initial flow rate).

During the formation of grains, pAg and pH were controlled by the use of potassium bromide aqueous solution and a 56% acetic acid aqueous solution. After the formation of grains, the grains were washed with water by a conventional flocculation method. Following this, gelatin was added thereto and for re-dispersion. At 40° C., the pH and pAg were respectively regulated to 5.8 and 8.06.

The resulting emulsion was a mono-dispersed emulsion containing an octahedral silver bromoiodide grains wherein an average grain size was 0.80  $\mu\text{m}$ , the width of grain size distribution was 12.4% and the silver iodide content was 8.5 mol %.

<G-1>

|                                              |         |
|----------------------------------------------|---------|
| Oscin gelatin                                | 100.0 g |
| Compound I (10% methanol solution by weight) | 25.0 ml |

**43**  
-continued

Ammonia (28% aqueous solution by weight) 440.0 ml  
Acetic acid (56% aqueous solution by weight) 660.0 ml  
Add water to make 5000.0 ml in total.  
<H-1>

Osein gelatin 82.4 g  
Potassium bromide 151.6 g  
Potassium iodide 90.6 g  
Add water to make 1030.5 ml in total.  
<S-1>

Silver nitrate 309.2 g  
Ammonia (28% aqueous solution by weight) Equivalent  
Add water to make 1030.5 ml in total.  
<H-2>

Osein gelatin 302.1 g  
Potassium bromide 770.0 g  
Potassium iodide 33.2 g  
Add water to make 3776.8 ml in total.

**44**  
-continued

5 <S-2>  
Silver nitrate  
Ammonia (28% aqueous solution by weight)  
Add water to make 3776.8 ml in total.

1133.0 g  
Equivalent

In the same manner as above, the average grain size of seed crystal, temperature, pAg, pH, flow rate, addition time and halide composition were changed so that the above-mentioned emulsions having different average grain size and silver iodide content were prepared. All emulsions were a core/shell type mono-dispersed emulsion wherein the variation coefficient of grain size distribution was 20% or less.

10 Each emulsion was subjected to the optimum chemical ripening in the presence of sodium thiosulfate, chloroaurate and ammonium thiocyanate wherein a sensitizing dye, 4-hydroxy- 6-methyl-1,3,3a,7-tetrazaindene and 1-phenyl-5-mercaptop tetrazole were added.



**45**

-continued

**46**

CC-1



CM-1



D-1



D-2



UV-1



UV-2



S-1



S-2



S-3



S-4



S-5



S-6

**49****50**

-continued

S-7



S-8



S-9



S-10



S-11



HS-1



HS-2

a mixture of



SC-1



Oil-1



Oil-2



Oil-3

-continued



$$(\text{CH}_2=\text{CHSO}_2\text{CH}_2)_2-\text{O}$$

H-1

H-2



$$\begin{array}{c} \text{H} \\ | \\ \text{NaO}_3\text{S} - \text{C} - \text{COOC}_8\text{H}_{17} \\ | \\ \text{CH}_2 - \text{COOC}_8\text{H}_{17} \end{array}$$

SU-1



AI-1



AI-2



ST-1



AE 1



AF-2



### Compound A

(Weight average molecular weight = 30,000)



## Replenisher for fixer

|                                   |        |
|-----------------------------------|--------|
| Water                             | 800 ml |
| Ammonium thiocyanate              | 150 g  |
| Ammonium thiosulfate              | 180 g  |
| Sodium sulfite                    | 20 g   |
| Ethylene diamine tetraacetic acid | 2 g    |

After pH was regulated to 6.5 using an aqueous ammonia solution or glacial acetic acid were used, water was added to make 1 liter in total.

## Stabilizer and replenisher for stabilizer

|                                                                                   |        |
|-----------------------------------------------------------------------------------|--------|
| Water                                                                             | 900 ml |
| The following compound No. 31                                                     | 2.0 g  |
| Compound 31                                                                       |        |
|  |        |
| Dimethylol urea                                                                   | 0.5 g  |
| Hexamethylene tetramine                                                           | 0.2 g  |
| 1,2-benzisothiazoline-3-on                                                        | 0.1 g  |
| Siloxane (L-77 produced by UCC)                                                   | 0.1 g  |
| Ammonia (aqueous solution)                                                        | 0.5 ml |

Water was added to make 1 liter in total, and pH was regulated to 8.5 using ammonia (aqueous solution) or a 50% sulfuric acid.

The maximum magenta color density of each sample subjected to photographic processing was measured by the use of a green light using an optical densitometer PDA-65 (produced by KONICA CORPORATION). Table 2 shows the maximum color density and relative sensitivity. In addition, Samples 201 through 213 were left for 5 days at 55° C., and then subjected to exposure to light and development so that the magenta density was measured. Table 7 shows the relative sensitivity.

TABLE 7

| Sample     | Magenta coupler | Maximum density | Relative sensitivity (1) | Relative sensitivity (2) left for 5 days at 55° C. |
|------------|-----------------|-----------------|--------------------------|----------------------------------------------------|
| 201 (Comp) | M-1             | 2.40            | 100                      | 100                                                |
| 202 (Inv)  | (1)             | 2.61            | 113                      | 121                                                |
| 203 (Inv)  | (2)             | 2.73            | 124                      | 144                                                |
| 204 (Inv)  | (9)             | 2.59            | 114                      | 140                                                |
| 205 (Inv)  | (12)            | 2.68            | 121                      | 141                                                |
| 206 (Inv)  | (14)            | 2.53            | 112                      | 138                                                |
| 207 (Inv)  | (22)            | 2.72            | 124                      | 145                                                |
| 208 (Inv)  | (24)            | 2.51            | 112                      | 130                                                |
| 209 (Inv)  | (28)            | 2.54            | 117                      | 149                                                |
| 210 (Inv)  | (29)            | 2.63            | 122                      | 142                                                |
| 211 (Inv)  | (30)            | 2.73            | 126                      | 142                                                |
| 212 (Inv)  | (32)            | 2.50            | 115                      | 122                                                |
| 213 (Inv)  | (33)            | 2.56            | 117                      | 132                                                |

The relative sensitivity (1) in Table 7 is a relative value of the inverse of an exposure amount giving the fog density+ 0.10 density value. Its value is represented by a relative value for the value of Sample 201 which is defined to be 100. In the same manner, relative sensitivity (2) is a relative value for the Sample 101 which is left for 5 days at 55° C. is defined to be 100.

As is apparent from Table 7, it can be understood that Samples 202 through 213 each using the magenta coupler of

the present invention are noticeably excellent compared to comparative sample 201 in terms of the maximum density, sensitivity and storage stability.

What is claimed is:

1. A silver halide color photographic light-sensitive material comprises a support having provided thereon at least one green-sensitive silver halide emulsion layer containing at least one of magenta coupler represented by Formula I or II:



wherein R<sup>1</sup> and R<sup>4</sup> each represent a substituent; R<sup>2</sup> and R<sup>3</sup> each represent a substituted or unsubstituted alkyl group; L<sub>1</sub> and L<sub>2</sub> each represent a substituted or unsubstituted alkylene group, an arylene group, an aralkylene group or an arylenealkylene group; Y represents



30 R<sup>5</sup> and R<sup>6</sup> each represent a substituent; X<sub>1</sub> represents a hydrogen atom or a group capable of splitting off upon reacting with an oxidized product of a color developing agent; Z represents non-metal atomic group forming a 5-membered or 6-membered heterocyclic ring together with a nitrogen atom; m and n each represent an integer of 0 or 1; p represents an integer of 0 to 4; q represents an integer of 0 to 2, provided that when p is 2 or more, R<sup>4</sup> may be the same or different; and each of them may form a ring.

35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 82

cycloalkyl group or an aryl group;  $R_{32}$  represents a halogen atom, an alkyl group, an alkenyl group, a cycloalkyl group or an aryl group; and  $n^2$  is an integer of 0 to 3; provided that, when two or more each of  $R_{31}$  and  $R_{32}$  are present, they may be the same with or the different from each other.  $Y_1$  represents S, SO, SO<sub>2</sub> or an alkylene group.

3. The material of claim 1, wherein said magenta coupler is Formula I:



Formula I

10  
15

wherein  $R^1$  and  $R^4$  each represent a substituent;  $R^2$  and  $R^3$  each represent a substituted or unsubstituted alkyl group;  $L_1$  and  $L_2$  each represent a substituted or unsubstituted alkylene group, an arylene group, an aralkylene group or an arylenealkylene group;  $Y$  represents

30  
35

$R^5$  and  $R^6$  each represent a substituent;  $X_1$  represents a hydrogen atom or a group capable of splitting off upon reacting with an oxidized product of a color developing agent;  $Z$  represents non-metal atomic group forming a 5-membered or 6-membered heterocyclic ring together with a nitrogen atom;  $m$  and  $n$  each represent an integer of 0 or 1;  $p$  represents an integer of 0 to 4;  $q$  represents an integer of 0 to 2, provided that when  $p$  is 2 or more,  $R^4$  may be the same or different; and each of them may form a ring.

4. The material of claim 3, wherein said material comprises an image-stabilizer represented by Formula A or B:



Formula A

55

wherein  $R_{21}$  represents a hydrogen atom, an alkyl group, an alkenyl group, an aryl group or a heterocyclic group;  $R_{22}$ ,  $R_{23}$ ,  $R_{25}$  and  $R_{26}$  each represent a hydrogen atom, a halogen atom, a hydroxyl group, an alkyl group, an alkenyl group, an aryl group, an alkoxy group or an acylamino group;  $R_{24}$  represents an alkyl group, a hydroxyl group, an aryl group, an alkoxy group, an alkenyloxy group or an aryloxy group;



Formula B

wherein  $R_{31}$  represents a secondary or tertiary alkyl group, a secondary or tertiary alkenyl group, a cycloalkyl group or an aryl group;  $R_{32}$  represents a halogen atom, an alkyl group, an alkenyl group, a cycloalkyl group or an aryl group; and  $n^2$  is an integer of 0 to 3; provided that, when two or more each of  $R_{31}$  and  $R_{32}$  are present, they may be the same with or the different from each other.  $Y_1$  represents S, SO, SO<sub>2</sub> or an alkylene group.

5. The material of claim 1, wherein said magenta coupler is Formula II:



Formula II

wherein  $R^1$  and  $R^4$  each represent a substituent;  $R^2$  and  $R^3$  each represent a substituted or unsubstituted alkyl group;  $L_1$  and  $L_2$  each represent a substituted or unsubstituted alkylene group, an arylene group, an aralkylene group or an arylenealkylene group;  $Y$  represents



$R^5$  and  $R^6$  each represent a substituent;  $X_1$  represents a hydrogen atom or a group capable of splitting off upon reacting with an oxidized product of a color developing agent;  $Z$  represents non-metal atomic group forming a 5-membered or 6-membered heterocyclic ring together with a nitrogen atom;  $m$  and  $n$  each represent an integer of 0 or 1;  $p$  represents an integer of 0 to 4;  $q$  represents an integer of 0 to 2, provided that when  $p$  is 2 or more,  $R^4$  may be the same or different; and each of them may form a ring.

6. The material of claim 5, wherein said material comprises an image-stabilizer represented by Formula A or B:



Formula A

wherein  $R_{21}$  represents a hydrogen atom, an alkyl group, an alkenyl group, an aryl group or a heterocyclic group;  $R_{22}$ ,  $R_{23}$ ,  $R_{25}$  and  $R_{26}$  each represent a hydrogen atom, a halogen atom, a hydroxyl group, an alkyl group, an alkenyl group, an aryl group, an alkoxy group or an acylamino group;  $R_{24}$  represents an alkyl group, a hydroxyl group, an aryl group, an alkoxy group, an alkenyloxy group or an aryloxy group;

59



Formula B

60

group is selected from the group consisting of



5

8. The material of claim 1, wherein said  $R^1$  of said Formula I or said Formula II is an alkyl group having 1 to 10 carbon atoms or an aryloxy group, and said



wherein  $R_{31}$  represents a secondary or tertiary alkyl group, a secondary or tertiary alkenyl group, a cycloalkyl group or an aryl group;  $R_{32}$  represents a halogen atom, an alkyl group, an alkenyl group, a cycloalkyl group or an aryl group; and  $n^2$  is an integer of 0 to 3; provided that, when two or more each of  $R_{31}$  and  $R_{32}$  are present, they may be the same with or the different from each other.  $Y_1$  represents S, SO, SO<sub>2</sub> or an alkylene group.

7. The material of claim 1, wherein said  $R^1$  of said Formula I or said Formula II is an alkyl group having 1 to 32 carbon atoms or an aryloxy group, and said



15

20

group is selected from the group consisting of



25

and said  $X_1$  is a halogen atom.

\* \* \* \* \*